

# United States Patent Office

3,226,328

Patented Dec. 28, 1965

1

3,226,328

## METHOD FOR MAKING LITHIUM NICKEL FERRITE HAVING A SUBSTANTIALLY RECTANGULAR HYSTERESIS LOOP

Cornelis Jacobus Esveldt, Ringenier Fluks, and Hans Peter Peloscheck, Emmasingel, Eindhoven, Netherlands, assignors to North American Philips Company, Inc., New York, N.Y., a corporation of Delaware

No Drawing. Filed Jan. 4, 1963, Ser. No. 249,339

Claims priority, application Netherlands, Jan. 5, 1962, 273,242

4 Claims. (Cl. 252—62.5)

Our invention relates to a ferromagnetic body having a substantially rectangular hysteresis loop for use as a memory element, and to a method of manufacturing such a body. Memory elements are used, for example, in electronic computers.

It is desirable to restrict the occurrence of eddy currents in memory elements as much as possible. Consequently, increasing use is made of ferromagnetic soft oxidic materials, which as is known, have a very small electric conductivity.

The utility of such cores as memory elements is based upon a significant difference between the "zero signal" and the "one signal" (in the computer technology the "zero" or "undisturbed" one signal,  $uV1$ , is distinguished from the "one" or "disturbed" one signal,  $rV1$ ; however, in a good memory element these quantities differ only slightly from one another). Consequently, it is necessary, in addition to sufficient "rectangularity" of the hysteresis loop that, for a given rise time of the control current, the lapse of time between the beginning of the control current pulse and the point of time at which the output voltage of the "one" signal reaches a strength of 10% of its maximum value is substantially constant. The "peak time" ( $T_p$ ) of a magnetic core is understood to mean the lapse of time between the point of time at which the control current reaches a strength of 10% of its maximum value and the point of time at which the output voltage of the "one" signal, which is produced by a control current pulse, has become a maximum. The peak time naturally depends upon the rise time ( $\tau_r$ ) of the control current pulse. Preferably the rise time should always be about 0.15 micro-second.

Variations in the current pulse characteristics of memory elements which occur as a result of temperature variations have thus far in most cases been corrected by varying the strength of the control current. Alternatively, the whole system of memory elements has been placed in a temperature-controlled environment to prevent disturbing temperature variations. However, these methods are complicated and cumbersome. In addition, they are useless if during operation of the system temperature differences occur between the individual memory elements because one element is switched a greater number of times in a given lapse of time than the other. It, therefore, is of great importance to have memory elements which not only have a sufficiently large squareness ratio, but also for which the output voltage of the "one" signal, and also the peak time, are only slightly dependent on the temperature over a wide temperature range (preferably between  $-50^\circ$  C. and  $+120^\circ$  C.).

It is an object of our invention to provide a ferromagnetic body having a substantially rectangular hysteresis loop for use as a memory element.

It is a further object of our invention to provide a new and novel ferromagnetic ferrite which exhibits a substantially rectangular hysteresis loop which is substantially less temperature dependent.

Another object of our invention is to provide a ferromagnetic ferrite body suitable for use as a memory

2

element which has a peak rise time substantially independent of temperature over a wide range of temperatures.

These and further objects of our invention will appear as the specification progresses.

In accordance with the invention, we have found that ferromagnetic bodies having a substantially rectangular hysteresis loop and which have peak rise times substantially independent of temperature over a wide range of temperatures when used as memory cores can be manufactured by mixing lithium oxide, nickel oxide, and ferric oxide in the proportions of about 2 to 20 mol percent of  $\text{Li}_2\text{O}$ , about 0.5 to 45 mol percent  $\text{NiO}$ , and about 50 to 85 mol percent  $\text{Fe}_2\text{O}_3$ , and after compacting the mixture to form a body, heating the mixture at a temperature of about  $1200^\circ$  to  $1400^\circ$  C. in an atmosphere containing at least as much oxygen as air.

In addition to the constituents  $\text{Li}_2\text{O}$ ,  $\text{NiO}$  and  $\text{Fe}_2\text{O}_3$  the mixture may also include up to 3 mol percent of  $\text{ZnO}$ , and up to 8 mol percent  $\text{CuO}$ . Further, instead of oxides of these metals, compounds which are converted by heating into oxides may be used. In order to insure a more homogeneous product, it may be desirable to reduce the heated product, after cooling, to a powder and reheating. The product may be reduced to powder several times and heated several times.

In a preferred embodiment, the mixture is heated at a temperature of about  $1200^\circ$  to  $1400^\circ$  C. after which it is first cooled at a rate of not more than  $30^\circ$  C. per minute to a temperature which is  $100^\circ$  to  $600^\circ$  C. below the heating temperature and is then quenched or, if the mixture which is heated at a temperature of about  $1200^\circ$  to  $1400^\circ$  C. is cooled at a rate of more than  $30^\circ$  C. per minute to a temperature which is  $100^\circ$  to  $600^\circ$  C. below the heating temperature, is maintained at this lower temperature for at least five minutes and then quenched.

The preferred composition of the cores for which optimum properties may be realized is in a range of compositions in which the oxides of lithium, nickel and iron correspond to

40      14-15 mol percent  $\text{Li}_2\text{O}$ ,  
5-7 mol percent  $\text{NiO}$ , and  
78-80 mol percent  $\text{Fe}_2\text{O}_3$ .

It should be noted that although lithium-nickel ferrite cores having a substantially rectangular hysteresis loop are known which are manufactured by heating at a temperature of from  $1100^\circ$  to  $1200^\circ$  C., they are less suitable as memory elements than those manufactured according to the present invention. More particularly, when used as memory cores, the difference between the output voltage of the "zero" signal and that of the "one" signal is significantly smaller. It was believed heretofore that the volatility of the lithium oxide handicapped the use of heating temperatures higher than  $1200^\circ$  C. It has appeared, however, that this is not the case provided that it is ensured that the sintering takes place in a gas atmosphere which contains very little, if any, water vapour.

The following examples are illustrations of the invention which is defined in the appended claims.

60      Mixtures of lithium carbonate,  $\text{Li}_2\text{CO}_3$ , nickel carbonate,  $\text{NiCO}_3$ , iron oxide,  $\text{Fe}_2\text{O}_3$ , and, if desired, zinc oxide,  $\text{ZnO}$ , and copper oxide,  $\text{CuO}$  were ground in ethanol in a ball mill for four hours. The ground products were presintered in air, cooled to room temperature and ground in ethanol in a ball mill for 16 hours. The resulting ground products, after the addition of an organic binding agent, were granulated and compacted into rings, at a pressure of  $1.5 \text{ ton/cm}^2$ , having an outside diameter of 1.63 mm., an inside diameter of 0.94 mm., and a height of 0.38 mm. These rings were heated in air by heating at a temperature between  $1200^\circ$  C. and  $1400^\circ$  C.

65      In some cases the pre-sintering was omitted. The fol-

lowing table specifies further details concerning the chemical composition and the conditions of preparing the cores as well as a number of measured results. The output voltage of the zero signal and that of the disturbed one signal ( $rV1$ ), as well as the peak time ( $T_p$ ) at a rise time ( $\tau_r$ ) of the control current pulse of 0.15 micro-second are specified for all compositions. All the measurements were carried out at 25° C. For some cores, the temperature coefficients of the undisturbed one signal ( $uV1$ ) and of the peak time ( $T_p$ ) are also specified.

2. A method of manufacturing a ferromagnetic body having a substantially rectangular hysteresis loop comprising the steps, forming a finely-divided mixture of about 2 to 20 mol percent of  $Li_2O$ , about 0.5 to 45 mol percent  $NiO$ , about 50 to 85 mol percent  $Fe_2O_3$ , up to 3 mol percent of  $ZnO$ , and up to 8 mol percent of  $CuO$ , compacting said mixture into a body, heating said body to a temperature of about 1200° to 1400° C. in an atmosphere substantially free of water-vapor containing at least as much oxygen by volume as air, cooling said body from said

TABLE I

| Core No. | Composition in mol percents of the oxides |       |       |       |           | Presintering temperature (° C.) | Way of sintering and cooling                                                                                                                      |
|----------|-------------------------------------------|-------|-------|-------|-----------|---------------------------------|---------------------------------------------------------------------------------------------------------------------------------------------------|
|          | $Li_2O$                                   | $NiO$ | $ZnO$ | $CuO$ | $Fe_2O_3$ |                                 |                                                                                                                                                   |
| 1        | 15.43                                     | 5.35  |       |       | 79.22     | 800                             | Passed through the furnace at a rate of 2 cm. per minute. In the heating zone of the furnace, 8 cms. long, a temperature of 1,243° C. prevailed.  |
| 2        | 14.55                                     | 6.45  |       |       | 79.0      | 750                             | Passed through the furnace at a rate of 2 cm. per minute. In the heating zone of the furnace, 8 cms. long, a temperature of 1,250° C. prevailed.  |
| 3        | 15.76                                     | 4.04  |       |       | 80.2      | 800                             | Heated at 1,255° C. for 10 minutes, cooled within the furnace to 1,000° C. and then quenched.                                                     |
| 4        | 16.3                                      | 1.2   |       |       | 82.5      | 750                             | Heated at 1,340° C. for 5 minutes, cooled within the furnace to 900° C. and then quenched.                                                        |
| 5        | 14.55                                     | 6.45  |       |       | 79.0      | 750                             | Heated at 1,340° C. for 10 minutes, cooled within the furnace to 1,000° C. and then quenched.                                                     |
| 6        | 14.55                                     | 6.45  |       |       | 79.0      | 625                             | Heated at 1,280° C. for 5 minutes, rapidly cooled to 980° C., maintained at 980° C. for 15 minutes and then quenched.                             |
| 7        | 14.55                                     | 6.45  |       |       | 79.0      |                                 | Heated at 1,340° C. for 5 minutes, cooled within the furnace to 1,000° C. and then quenched.                                                      |
| 8        | 14.55                                     | 6.45  |       |       | 79.0      |                                 | Heated at 1,350° C. for 5 minutes, rapidly cooled to 1,020° C., maintained at 1,020° C. for 10 minutes and then quenched.                         |
| 9        | 14.55                                     | 5.45  | 1.0   |       | 79.0      | 775                             | Heated at 1,337° C. for 5 minutes, cooled within the furnace to 1,000° C. and then quenched.                                                      |
| 10       | 14.55                                     | 4.45  | 2.0   |       | 79.0      | 775                             | Heated at 1,350° C. for 5 minutes, rapidly cooled to 1,100° C., maintained at 1,100° C. for 40 minutes and then quenched.                         |
| 11       | 8.8                                       | 17.7  |       |       | 5.9       | 750                             | Heated at 1,340° C. for 5 minutes, cooled within the furnace to 970° C. and then quenched.                                                        |
| 12       | 12.5                                      | 6.25  |       |       | 6.25      | 750                             | Heated at 1,262° C. for 7 minutes, rapidly cooled to 970° C., maintained at 970° C. for 15 minutes and then quenched.                             |
| 13       | 15.03                                     | 5.23  |       |       | 79.74     | 900                             | Passed through the furnace at a rate of 2 cms. per minute. In the heating zone of the furnace, 8 cms. long, a temperature of 1,235° C. prevailed. |
| 14       | 15.43                                     | 5.35  |       |       | 79.22     | 800                             | Heated at 1,218° C. for 10 minutes, cooled within the furnace to 1,050° C. and then quenched.                                                     |

TABLE II.—MEASURED RESULTS

| Core No. | Output voltage of the zero signal (millivolts) | Output voltage of the disturbed one signal, $rV1$ (millivolts) | Peak time, $T_p$ (micro-seconds) | Temperature coefficient of the peak time, $T_p$ |                          | Temperature coefficient of the undisturbed one signal, $uV1$ |                          |
|----------|------------------------------------------------|----------------------------------------------------------------|----------------------------------|-------------------------------------------------|--------------------------|--------------------------------------------------------------|--------------------------|
|          |                                                |                                                                |                                  | Percent per ° C.                                | In the temp. range from— | Percent per ° C.                                             | In the temp. range from— |
| 1        | 14                                             | 42                                                             | 0.33                             | 0.0                                             | +25° C. to +60° C.       | 0.56                                                         | +25° C. to +60° C.       |
| 2        | 32                                             | 85                                                             | 0.58                             |                                                 |                          | 0.6                                                          | +20° C. to +60° C.       |
| 3        | 13                                             | 48                                                             | 9.43                             | 0.0                                             | +20° C. to +60° C.       |                                                              |                          |
| 4        | 14                                             | 64                                                             | 0.44                             |                                                 |                          | 0.53                                                         | -40° C. to +160° C.      |
| 5        | 18                                             | 94                                                             | 0.33                             | 0.0                                             | -40° C. to +140° C.      |                                                              |                          |
| 6        | 25                                             | 108                                                            | 0.27                             |                                                 |                          |                                                              |                          |
| 7        | 29                                             | 114                                                            | 0.26                             |                                                 |                          |                                                              |                          |
| 8        | 36                                             | 118                                                            | 0.25                             |                                                 |                          |                                                              |                          |
| 9        | 14                                             | 61                                                             | 0.6                              | 0.0                                             | -10° C. to +100° C.      | 0.55                                                         | -40° C. to +160° C.      |
| 10       | 18                                             | 40                                                             | 0.5                              |                                                 |                          |                                                              |                          |
| 11       | 95                                             | 225                                                            | 0.23                             |                                                 |                          |                                                              |                          |
| 12       | 110                                            | 230                                                            | 0.22                             |                                                 |                          |                                                              |                          |
| 13       | 14                                             | 31                                                             | 0.3                              | 0.0                                             | +20° C. to +60° C.       | 0.46                                                         | +20° C. to +60° C.       |
| 14       | 15                                             | 48                                                             | 0.44                             | 0.0                                             | +20° C. to +60° C.       | 0.49                                                         | +20° C. to +60° C.       |

While we have described our invention in connection with specific embodiments and applications thereof, other modifications will thus be apparent to those skilled in the art without departing from the spirit and scope of the invention as defined in the appended claims.

What we claim is:

1. A method of manufacturing a ferromagnetic body having a substantially rectangular hysteresis loop comprising the steps, forming a finely-divided mixture of about 2 to 20 mol percent of  $Li_2O$ , about 0.5 to 45 mol percent  $NiO$ , about 50 to 85 mol percent  $Fe_2O_3$ , up to 3 mol percent of  $ZnO$ , and up to 8 mol percent of  $CuO$ , compacting said mixture into a body, heating said body to a temperature of about 1200° to 1400° C. in an atmosphere substantially free of water-vapor containing at least as much oxygen by volume as air, cooling said body from said heating temperature to a temperature of about 100° to 600° C. below the heating temperature at a rate of not more than 30° C. per minute, and quenching said body from the temperature to which it was cooled.

60 heating temperature to a temperature which is 100° to 600° C. lower than said heating temperature at a rate which is greater than 30° C. per minute maintaining said body at said latter temperature for at least five minutes, and quenching said body from said latter temperature.

3. A method of manufacturing a ferromagnetic body having a substantially rectangular hysteresis loop comprising the steps, forming a finely-divided mixture of about 14 to 15 mol percent of  $Li_2O$ , about 5 to 7 mol percent  $NiO$ , about 78 to 80 mol percent  $Fe_2O_3$ , compacting said mixture into a body, heating said body to a temperature of about 1200° to 1400° C. in an atmosphere substantially free of water-vapor and containing at least as much oxygen by volume as air, cooling said body from said heating temperature to a temperature about 100° to 600° C. below said heating temperature at a rate of not more than 30° C. per minute, and quenching said body from said latter temperature.

4. A method of manufacturing a ferromagnetic body having a substantially rectangular hysteresis loop com-

prising the steps, forming a finely-divided mixture of about 14 to 15 mol percent of  $\text{Li}_2\text{O}$ , about 4 to 7 mol percent  $\text{NiO}$ , about 78 to 80 mol percent  $\text{Fe}_2\text{O}_3$ , compacting said mixture into a body, heating said body to a temperature of about  $1200^\circ$  to  $1400^\circ$  C. in an atmosphere substantially free of water-vapor and containing at least as much oxygen by volume as air, cooling said body from said heating temperature to a temperature about  $100^\circ$  to  $600^\circ$  C. below said heating temperature at a rate greater than  $30^\circ$  C. per minute, maintaining said body at said latter temperature for at least five minutes,

and quenching said body from said latter temperature.

References Cited by the Examiner

UNITED STATES PATENTS

- |   |           |        |               |       |          |
|---|-----------|--------|---------------|-------|----------|
| 5 | 2,882,234 | 4/1959 | Gorter et al. | ----- | 252—62.5 |
|   | 3,033,792 | 5/1962 | Kikuchi       | ----- | 252—62.5 |
|   | 3,038,860 | 6/1962 | Vinal et al.  | ----- | 252—62.5 |

TOBIAS E. LEVGW, *Primary Examiner.*

10 MAURICE A. BRINDISI, *Examiner.*